

July 25, 1933.

M. O. SCHUR ET AL

1,919,962

CONDITIONING OF CELLULOSE FIBER FOR NITRATION

Filed Feb. 20, 1930



Inventor:  
Milton O. Schur,  
Benjamin G. Hoos.  
by Wright, Brown, Quincy & May  
Attns.

Patented July 25, 1933

1,919,962

# UNITED STATES PATENT OFFICE

MILTON O. SCHUR AND BENJAMIN G. HOOS, OF BERLIN, NEW HAMPSHIRE, ASSIGNOR  
TO BROWN COMPANY, OF BERLIN, NEW HAMPSHIRE, A CORPORATION OF MAINE

## CONDITIONING OF CELLULOSE FIBER FOR NITRATION

Application filed February 20, 1930. Serial No. 429,926.

This invention relates to the conditioning of cellulose fiber for conversion into cellulose derivatives. It deals more especially with the conditioning of cellulose fiber of the nature of wood pulp for nitration, with a view toward enhancing the qualities and the yield of nitrocellulose attainable from the fiber used as raw material.

In the cellulose derivative industry, considerable attention is paid to both the chemical and physical characteristics of the cellulose fiber to be converted into derivatives. This is particularly true in the field of nitration, where it is essential that the cellulose fiber not only answer certain specifications as to composition, but that it also be in such physical condition that nitration will proceed with smoothness, uniformity, and minimum side reaction and will result in a high yield of nitrate of good quality and low acid retention.

In our application Serial No. 394,370, Patent No. 1,880,052, the discovery was announced that when cellulose fiber is finely shredded under predetermined conditions of moisture content, and then dried, it takes on a physical condition highly satisfactory for nitration, as attested by the favorable progress of nitration and the high yield of nitrate of good quality. We have now discovered that additional striking advantages may be realized if the fiber is in mercerized as well as in moist condition during the shredding operation. These advantages include a still higher yield of nitrated product, a lower acid retention, and at the same time the opportunity of carrying out the shredding operation within wider limits of moisture in the fiber and with a variety of available shredding machines. Mercerization evidently so changes the physical character of the fiber that it is easy to avoid the generation of fibrous dust while shredding at low moisture contents, as well as to do away with hard-packed lumps while shredding at high moisture contents. While some shredding machines lead to better results than others, with a given machine far better results are obtained in the case of a mercerized fiber than in the case of similar

unmercerized fiber. For instance, an impact shredding machine, such as a hammer mill, which leads to eminently satisfactory results in the case of a mercerized fiber, must be carefully adjusted and controlled in order to lead to good results in the case of similar unmercerized fiber. The shredding of the mercerized fiber may be practiced to especial advantage with a hammer mill, as such a machine is rugged and comparatively inexpensive, and has a high output of product. The mercerized fiber may, however, be shredded by the use of other machines, such as carding machines, which sometimes lead to even higher yields of nitrate than that obtained when using a hammer mill.

While the process of the present invention may be practised to advantage upon various cellulose fibers, it is especially worth while in the case of wood pulps, such as the refined wood pulps of high alpha cellulose content, which offer greater opportunity for improvement than cotton linters, which has heretofore constituted practically the only satisfactory source of cellulose for nitration. A major advantage of our process is that the finely shredded, mercerized wood fiber may be handled by the nitration manufacturer, who has been in the custom of using cotton linters, with no fundamental change in the process or the instrumentalities with which he is equipped. Thus, should the nitration mill be at a point distant from where mercerization and shredding is performed, the dried shreds may be shipped to the nitration mill in bales, as is cotton linters. Should the nitration mill be one in which so-called lower nitrocelluloses, e. g., those of 11% nitrogen content, are made, the procedure may be one which is typical in such case. Such a procedure may be substantially as follows. Care is initially taken that the shreds are in dry condition before their addition to the nitrating pots. The dry shreds are steeped in a nitrating acid mixture comprising 18.7% water, 20.5% nitric acid, and 60.8% sulphuric acid, the ratio of acid to fiber being 50 to 1. The

temperature of the reacting charge is regulated according to the viscosity of the nitro-cellulose desired, a typical nitration being carried out at 40° C. for one-half hour. At 5 the end of nitration, the contents of the nitrating pot are dumped into a centrifuge, wherein the excess acid is whizzed off, and the centrifuged mass of shreds is pitch-forked into tanks wherein it is subjected to 10 high pressure streams of fresh water, which serve to dilute quickly residual acid associated with the centrifuged mass. The washed mass is drained free from excess water, is again washed and drained free 15 from excess water, and is then boiled in water under atmospheric pressure for from three to twenty-four hours, with one or more changes of water during the boiling operation. Boiling of the nitrated product serves 20 to remove traces of acid and impurities therefrom, and thus to effect its stabilization. The boiled product is washed with a large volume of cold water, and centrifuged to a low water content. The water in the 25 centrifuged product is displaced by denatured alcohol, and in this condition the product may be sold or compounded with other materials, such as camphor, to produce ultimate nitrocellulose products.

30 When subjected to the mercerizing step of our process, the cellulose fiber may be in any one of a variety of forms, depending upon the conditions at hand. For example, if mercerization is carried out in a pulp mill 35 where fiber is handled in slush form, the fiber is mercerized in such form, but if mercerization is to be effected in a nitration mill operating distant from a pulp mill and to which the fiber is shipped in the form of 40 comparatively thick sheets, such as used in viscose-rayon manufacture, in the form of paper or tissue, or in the form of shreds, the fiber may be mercerized in any one of these forms. The caustic soda solution used for 45 mercerizing the fiber may be at room temperature or at much lower temperature, depending upon the mercerizing temperature of the solution employed. For instance, when a caustic soda solution of 18% 50 strength is used, mercerization may be effected at room temperature, but if the caustic soda solution is of lower strength, say 10%, mercerization cannot be effected at above about 0° C. The time required for 55 mercerization is exceedingly short, being as low as two to three minutes, but, inasmuch as caustic soda solution extracts impurities from cellulose fiber, including less-resistant celluloses and ligneous and resinous matter, 60 it may be of advantage to maintain the fiber in contact with the solution for a substantial period of time, especially when unbleached or relatively impure pulps are used as raw material. If desired, other purifying chemicals, such as bleach, which tend to improve 65

the color of the fiber, may be present in the caustic soda solution. Other alkalis may be present in solution, along with the caustic soda. For instance, if mercerization is performed in a kraft mill where so-called white liquor, consisting of a solution of caustic soda and sodium sulphide, is available, such a liquor may be utilized for mercerizing the fiber. When an unbleached, relatively impure pulp is used as raw material, it may be subjected to chemical refining steps such as chlorination, bleaching and/or high temperature cooking in dilute liquors before or after mercerization.

When the fiber requires mercerization as the only chemical treatment prior to the shredding operation, it is washed immediately after mercerization and is preferably acidified toward the completion of washing with dilute acid, such as acetic or sulphurous, to ensure complete removal of caustic soda. It is then necessary to dewater the mercerized fiber to the moisture content at which it may be shredded to the physical condition satisfactory for nitration. To this end, the pulp should be dewatered until it has a fiber content of from about 25% to 75%, but optimum results are obtainable at fiber contents of from about 30% to 65%. When the pulp has been mercerized and washed in the form of comparatively thick sheets, they may be dewatered under action of hydraulic presses to a fiber content as high as about 40%. If, however, the pulp is mercerized and washed in the form of a suspension of individual fibers or shreds, dewatering may be effected by sheeting on a wet or cylinder machine equipped with sufficiently heavy couch and pressure rolls to produce sheets of as high as about 25% fiber content. These sheets may then be dewatered under the action of hydraulic presses to higher fiber content. Or the mercerized and washed pulp suspension may be dewatered directly to a fiber content of about 40% by centrifuging. If higher than about 40% fiber is desired in the pulp, the partially dewatered pulp may be subjected to a drying operation, in which case drying should be conducted to ensure a product throughout which the moisture is uniformly distributed, as it is necessary that shredding be carried out on a uniformly moist material. When it is desired to carry a comparatively large stock of mercerized fiber or when mercerization is carried out at a much higher rate than shredding, and storing of mercerized fiber is necessary, the mercerized fiber should be dewatered to complete dryness in order to avoid deterioration of the pulp such as takes place when it is stored in moist condition for a long period. In such case, however, the dry, mercerized fiber should be uniformly rewetted to the desired moisture content before shredding.

We shall now describe a specific example of procedure falling within the purview of the present invention. The fiber employed as raw material was bleached, refined wood pulp of 93% alpha cellulose content, in the form of drier sheets of 95% fiber content. These sheets were steeped in a bath of 17.5% caustic soda solution at room temperature, say 18° to 20° C., and in which the ratio of solution to fiber was about 19 to 1 so as to ensure complete and uniform contact of the solution with all the fibers. The sheets were thoroughly pulped or suspended in the solution by agitation, and after about three 15 minutes the fiber suspension was thrown on a filter, the excess liquor drained off, and the mercerized fiber retained on the filter was thoroughly washed with hot water, which tends to enhance the purification of 20 the fiber. The fiber was then acidified with a weak solution of acetic acid and again washed to remove last traces of chemical. The washed fiber was then centrifuged to a fiber content of about 30%, was coarsely 25 shredded, and air-dried to a fiber content of about 50%. The fiber was then passed through a hammer mill, wherein it was finely shredded. The mass of shreds was brought to a bone-dry condition, in which 30 condition it had an appearance closely resembling cotton linters. When nitrated under the conditions hereinbefore described to produce nitrocellulose of 11% nitrogen content, and then centrifuged, the yield of product was 153.0 and the acid retention 5.3 or 35 1.7 pounds of spent nitrating acid per pound of nitrocellulose. These results are comparable to those obtained when using high grade cotton linters as a raw material.

40 The foregoing results are illustrative of those obtained when similar mercerized fiber is shredded under other conditions of moisture content and then completely dried and nitrated. On the accompanying drawing, 45 the nitrating yield and acid retention values obtained in the case of shredded, mercerized, refined wood pulp are plotted against the fiber content during shredding. It is to be noted that both the yield and acid retention 50 curves reach a maximum and minimum, respectively, at the region of about 30% to 65% fiber content, at which content we prefer to carry out the shredding operation, but even at as high a fiber content as 75% 55 and as low as 25%, we obtain good results.

While our discoveries may be applied to advantage in conditioning cellulose fibers of various origins for conversion into nitrocelluloses, they have especial significance 60 when applied to refined wood pulp of high alpha cellulose content, say of about 93% alpha cellulose content or higher. Such wood pulps are highly absorptive as a result of the removal of non-alpha cellulose impur-

ities therefrom, and when prepared in fluffed form, as ordinarily for nitration, give disappointing results. We believe that secondary reactions are encouraged when such wood fiber is fluffed, it being our theory that 70 as the mixed nitrating acids react with fiber, they become weaker in nitric acid and richer in water content, tending to hydrolyze the fibers rather than to nitrate them. Since the fibers are in a highly absorptive condition, nitration of the fibers evidently takes place so rapidly that there is insufficient time for diffusive action to take place to ensure the proper composition of mixed nitrating acids in the fibers. The disappointing 75 results originally obtained when using refined wood pulps are doubtless traceable to the additive effect of the absorptivity of the individual fibers, and the absorptivity of the mass. At the early stages of our research work, we were at a loss to account for these results, as one might expect good results because of the desirable chemical composition of the fiber. By conditioning such wood fiber as hereinbefore described, it is 80 possible to realize the good results to be expected from such fiber, without incurring such expense as to nullify the economical advantage which such fiber now has over cotton. 85

We claim:

1. A process which comprises suspending preliberated cellulose fiber in a large excess of caustic soda solution under mercerizing conditions, washing the mercerized fiber free 100 from alkaline solution, dewatering the washed fiber to a fiber content of from about 25% to 75%, shredding the fiber, completely drying the shreds while at such moisture content from such moist condition, and nitrating the resulting dried shreds. 105

2. A process which comprises shredding mercerized wood pulp while associated with water in amount to produce a fiber content of from about 25% to 75%, drying the shreds 110 from such moisture content, and nitrating the resulting dried shreds. 110

3. A process which comprises finely shredding a mass of mercerized cellulose pulp in the presence of moisture, drying the moist shreds, and nitrating the dried shreds. 115

4. A process which comprises mercerizing wood pulp, finely shredding the mercerized pulp in the presence of moisture, drying the shreds, and nitrating the dried shreds. 120

5. A process which comprises treating cellulose fiber with a mercerizing liquor, washing the fiber free from such liquor, removing water from the washed fiber until its moisture content is sufficiently low to permit fine-shredding, finely shredding the moist fiber, drying, and nitrating. 125

MILTON O. SCHUR.  
BENJAMIN G. HOOS.